

[54] **CELLULOSIC MATERIALS INTERNALLY SIZED WITH LOW MOLECULAR WEIGHT COPOLYMERS OF ALPHA, BETA-ETHYLENICALLY UNSATURATED HYDROPHOBIC MONOMERS AND AMMONIATED CARBOXYLIC ACID COMONOMERS**

[75] Inventors: **Walter Lee Vaughn**, Lake Jackson; **Robert James Beam**, Angleton, both of Tex.

[73] Assignee: **The Dow Chemical Company**, Midland, Mich.

[22] Filed: **Feb. 1, 1974**

[21] Appl. No.: **438,914**

[52] U.S. Cl. .... **260/17.4 ST**, 162/164, 162/168, 162/169, 162/175, 162/185, 260/17.4 CL

[51] Int. Cl. .... **C08g 45/18**

[58] Field of Search .... **260/17.4 ST, 17.4 CL; 162/168, 164, 175, 185, 169**

[56] **References Cited**

UNITED STATES PATENTS

3,279,975 10/1966 Yoshii et al. .... 162/168

|           |        |                   |         |
|-----------|--------|-------------------|---------|
| 3,575,796 | 4/1971 | Brown et al. .... | 162/158 |
| 3,655,506 | 4/1972 | Baggett ....      | 162/164 |
| 3,674,896 | 7/1972 | Purcell ....      | 260/897 |

OTHER PUBLICATIONS

Union Carbide Brochure, "F-42958," Products for Paper, PC4-300, Analkal: Dispersible Ethylene Copolymer, printed 10/70; pp. 1-2, 4-12, and 14.

Primary Examiner—Morris Liebman

Assistant Examiner—Edward Woodberry

Attorney, Agent, or Firm—Richard G. Waterman; Michael S. Jenkins

[57] **ABSTRACT**

Cellulosic materials such as paper are internally sized by treating fibers of the cellulosic material, e.g., paper pulp, with a low molecular weight copolymer of an  $\alpha, \beta$ -ethylenically unsaturated hydrophobic monomer and an ammoniated,  $\alpha, \beta$ -ethylenically unsaturated carboxylic acid and a cationic retention aid. Internal sizing of the cellulosic material by this method can be carried out under acidic, neutral or basic conditions.

**21 Claims, No Drawings**

**CELLULOSIC MATERIALS INTERNALLY SIZED  
WITH LOW MOLECULAR WEIGHT  
COPOLYMERS OF ALPHA,  
BETA-ETHYLENICALLY UNSATURATED  
HYDROPHOBIC MONOMERS AND AMMONIATED  
CARBOXYLIC ACID COMONOMERS**

**BACKGROUND OF THE INVENTION**

This invention relates to internal sizing of cellulosic material over the complete range of pH conditions which are normally encountered in the cellulosic manufacturing arts.

Cellulosic materials such as paper and paperboard, are often sized with various materials with the purpose of increasing their resistance to water penetration as well as to penetration by other types of aqueous solutions. These materials are referred to as sizes or sizing agents and they may be introduced during the actual manufacture of the cellulosic material, e.g., paper making operation, wherein the process is known as internal sizing, often called beater sizing, wet end sizing or engine sizing. Surface sizing cellulosic materials by applying sizing agent to fabricated sheet or web is also well known; but is usually considered to be substantially different from internal sizing.

The basis of present internal sizing methods is the intimate coating of the individual fibers of the cellulosic material with a material which is insoluble in most materials and is repellent to water. For example, in manufacture of paper, the substance originally and still most widely used for this purpose is rosin or fatty acid. In order to insure the most intimate contact between the rosin and the pulp fiber, the former is added in either the dissolved state or as a finely dispersed emulsion. It is followed by a precipitating agent, usually aluminum sulfate, known to the paper maker as "alum." The alum coagulates the rosin, i.e., throws it out of solution or emulsion as a gelatinous precipitate. Since the rosin or emulsion is first mixed thoroughly with the pulp in the beater, the precipitate has a maximum chance of adhering to and being subsequently retained by the pulp. When the pulp is made into paper, the rosin in contact with the pulp adheres to the pulp as small particles, e.g., particles having diameters of one micron or less. The paper having the small particles of rosin adhered to the fibers exhibits the desired strength and ink and water resistance.

In addition to rosins, various water-repellant or hydrophobic materials have been utilized as internal sizing agents. These include fortified rosin, mixtures or rosins with waxes, wax emulsions, ketone dimer emulsions, fluorocarbons, fatty acid complexes of chromium or aluminum chlorides, long chain thermoplastic copolymers, as well as thermosetting condensation-type resins. Although all of these materials are effective under certain conditions, their use is nonetheless subject to one or more limitations.

For example, in the case of rosin, it is only useful as sizing agent in acidic solutions and therefore cannot be used for the sizing of neutral or alkaline pulps. Rosin is inoperable with the latter since it must ordinarily be used in combination with alum, or an acidic aluminum ion donor which is present for the purpose of precipitating and setting the metal rosinate onto the fibers. The use of alum for this purpose is, however, precluded under neutral or alkaline stock conditions. This is a definite disadvantage in paper making since paper pro-

duced from neutral or alkaline pulp has been found to have higher strength, greater stability and superior aging characteristics in comparison with paper prepared from acidic pulp. Also, the internal use of alkaline pigments such as calcium carbonate is precluded. This limitation also applies to most wax emulsions which cannot be used on the alkaline side since they are usually combined with small quantities of alum for the purpose of breaking the emulsions. On the other hand, it may be noted that certain sizing agents will not tolerate acidic conditions. In addition to the above described pH limitations, the water resistance or water holdout which is obtainable with many of the heretofore employed sizing agents is often inadequate for many applications which require paper or paperboard displaying an exceptionally high degree of water-resistance. Some sizing agents provide complete water repellancy as opposed to the desired limited amount of water-resistance. Many sizing agents have been found to be incompatible with pigments, fillers or other ingredients which are often added to the paper. A further disadvantage of some sizing agents is that a considerable degree of heat curing is required in order to develop full effectiveness.

For these and other reasons, it would be highly desirable to provide an internal sizing agent which can be effectively employed under acidic, neutral or alkaline conditions and which can be cured to a size having the desired limited water resistance under normal drying conditions used in the early stages of manufacturing paper and other cellulosic materials.

**SUMMARY OF THE INVENTION**

In the present invention, paper and other cellulosic materials are internally sized under pH conditions ranging from moderately acidic through strongly alkaline by an improved internal sizing method. In this improved method for internally sizing the cellulosic material wherein an internal sizing agent is applied to the fibers of the cellulosic material, the improvement comprises the use of a low molecular weight copolymer of an  $\alpha,\beta$ -ethylenically unsaturated hydrophobic monomer and an ammoniated  $\alpha,\beta$ -ethylenically unsaturated carboxylic acid as an internal sizing agent and a cationic retention aid. In another aspect, this invention is an internal sizing composition for a cellulosic material comprising a sizing amount of the aforementioned copolymer and an amount of a cationic retention aid which is effective to retain the copolymer on the cellulosic material. In a further aspect, this invention is a cellulosic material internally sized with the aforementioned composition. The resultant internally sized cellulosic material displays a very desirable degree of water-resistance along with resistance of acidic and alkaline solutions. Of prime importance is the fact that the successful use of the aforementioned copolymers as sizing agents is not restricted to acidic pH which thus allows utilization of such sizing agents in the treatment of neutral and alkaline pulp as well as acidic pulp. Furthermore, it is found that only mild drying and curing conditions are needed to develop the full sizing value of such internal sizing agents.

**DETAILED DESCRIPTION OF THE INVENTION**

For the purposes of this invention, the term "cellulosic material" is meant to include paper, paper board and other fibrous, sheet-like or molded masses derived

from wood, wood pulp, or cotton or other sources of cellulosic fibers. This term also includes sheet-like or molded masses prepared from combination of cellulosic materials and non-cellulosic materials such as polyamides, polyesters, polyacrylic acid resin fibers and mineral fibers such as asbestos, glass and the like.

By the term "internal-sizing" is meant a method of sizing in which the cellulosic material in raw form, e.g., fibrous stock such as paper pulp, is contacted with the sizing agent under conditions effective to size the cellulosic material, i.e., deposit the sizing agent on the fibers and cure it to full sizing effectiveness. Accordingly, it is understood that the term "internal sizing" is generic, and therefore includes such terms as "beater-sizing," "engine-sizing," "internal wet end sizing" and the like.

The internal sizing agents suitably employed in the practice of this invention are copolymers of  $\alpha,\beta$ -ethylenically unsaturated hydrophobic monomer and ammoniated  $\alpha,\beta$ -ethylenically unsaturated carboxylic acid, i.e.,  $\alpha,\beta$ -ethylenically unsaturated carboxylic acid in the ammonium salt form. Generally, such copolymers are water-dispersible, semi-solid or solid materials. The molecular weights of such copolymers, measured as number average molecular weight by embulliometry, are suitably in the range generally from about 1,000 to about 10,000, preferably from about 3,000 to about 8,000 and especially from about 4,000 to about 7,000. Suitable copolymers have melt flow viscosities in the range generally from about 0.5 decigram/minute to about 50 decigrams/minute as measured using the procedure of ASTM D-1238-65T(B) except that the orifice of the extrusion plastometer is 0.020 inch. Preferably the copolymers are film-forming at temperatures used in the sizing operations. By "water-dispersible" is meant a material which can exist in the form of a stable aqueous colloidal dispersion in the absence of a surface active agent. In addition, the copolymers in the form of aqueous dispersion preferably form films under ambient conditions which films dry to form water-insoluble coatings. By  $\alpha,\beta$ -ethylenically unsaturated hydrophobic monomer is meant any water-immiscible monomer containing a terminal double bond capable of polymerization under normal conditions of addition polymerization to form a water-insoluble homopolymer having a polyethylenic backbone. By " $\alpha,\beta$ -ethylenically unsaturated carboxylic acid" is meant an  $\alpha,\beta$ -ethylenically unsaturated carboxylic acid which is capable of addition copolymerization through the ethylenically unsaturated group with the  $\alpha,\beta$ -ethylenically unsaturated hydrophobic monomer. By "ammoniated  $\alpha,\beta$ -ethylenically unsaturated carboxylic acid" is meant that in the copolymer the carboxylic acid groups are neutralized with ammonia.

Preferably, the internal sizing agent is a normally solid, water- and alkali-insoluble thermoplastic addition copolymer in the form of a fluid aqueous colloidal dispersion. The occurrence of ammoniated acid groups in the polymer should be general throughout the macromolecules thereof so that each macromolecule contains a minimum number of active salt groups sufficient to render the polymer water-dispersible as defined hereinbefore. The maximum number of ammoniated acid groups which may be present in the macromolecules is fixed by the requirement that the molecule be substantially water-insoluble. Generally speaking, such copolymers contain from about 6 to about 40 weight percent of ammoniated acid comonomer, with

preferred copolymers containing from about 10 to about 20 weight percent of ammoniated acid comonomer and especially preferred copolymers containing from about 15 to about 18 weight percent.

Exemplary preferred copolymers are the random copolymer products of copolymerization of mixtures of one or more polymerizable ethylenically unsaturated carboxylic acids having 3 to 8 carbon atoms inclusive of anhydrides and alkyl half esters of ethylenically unsaturated acids such as acrylic acid, methacrylic acid, maleic acid and anhydride, itaconic acid, fumaric acid, crotonic acid and citraconic acid and anhydride, methyl hydrogen maleate, ethyl hydrogen maleate, and one or more  $\alpha,\beta$ -ethylenically unsaturated hydrocarbon monomers such as the aliphatic  $\alpha$ -olefin monomers, e.g., ethylene, propylene, butene-1 and isobutene; conjugated dienes, e.g., butadiene and isoprene; and monovinylidene aromatic carbocyclic monomers, e.g., styrene,  $\alpha$ -methylstyrene, toluene, and t-butylstyrene. In addition, other ethylenically unsaturated hydrophobic monomers which are not entirely hydrocarbon are copolymerized with the aforementioned acid comonomers. Examples of such suitable monomers which are not entirely hydrocarbon include esters of  $\alpha,\beta$ -ethylenically unsaturated carboxylic acids such as ethyl acrylate, methyl methacrylate, ethyl methacrylate, methyl acrylate, isobutyl acrylate, and methyl fumarate; unsaturated esters of non-polymerizable carboxylic acids such as vinyl acetate, vinyl propionate, and vinyl benzoate; vinyl halides such as vinyl and vinylidene chloride; vinyl ethers;  $\alpha,\beta$ -ethylenically unsaturated amides and nitriles such as acrylamide, acrylonitrile, methacrylonitrile and fumaronitrile. It is understood that the aforementioned suitable hydrophobic monomers may be copolymerized with preferred hydrocarbon monomer and the acid comonomer in proportions such that a water- and alkali-insoluble polymer is provided. Preferred copolymers include copolymers from about 70 to about 90 weight percent of ethylene, from about 10 to about 20 weight percent of one or more ammoniated ethylenically unsaturated acids such as acrylic acid and methacrylic acid and from 0 to about 20 weight percent of suitable ethylenically unsaturated hydrophobic monomer as described hereinbefore such as acrylonitrile, ethyl acrylate and vinyl acetate.

Other copolymers which are suitable are made from pre-formed, non-acid polymers by subsequent chemical reactions carried out thereon. For example, the carboxylic acid group may be supplied by grafting a monomer such as acrylic acid or maleic acid onto a polymer substrate such as polyethylene. Additionally, copolymers containing carboxylic anhydride, ester, amide, acylhalide and nitrile groups can be hydrolyzed to carboxylic acid groups which can then be neutralized to form the ammoniated carboxylic acid.

It is further understood that the  $\alpha,\beta$ -ethylenically unsaturated carboxylic acid in ammonium salt form may be copolymerized with the hydrophobic monomer in order to prepare a suitable copolymer.

Specified procedures and means for making the polymers are known to the art as exemplified by U.S. Pat. No. 3,520,861 to Thomson et al. and U.S. Pat. No. 3,426,363 to Helin. The low molecular weight copolymers are advantageously prepared by employing a telogen such as propylene in the practice of the process of U.S. Pat. No. 3,520,861. In instances wherein the acid

copolymer is obtained in mass form, the copolymer may be converted to aqueous colloidal dispersion in accordance with the methods of U.S. Pat. No. 3,389,109 to Harmon, et al. which is subsequently concentrated and ammoniated by the method described in U.S. Pat. No. 3,644,258 to Moore et al. Generally methods of producing the aqueous colloidal dispersion of a copolymer which require the use of little or not emulsifier or other surface active agents are preferred. Preferably, the aqueous colloidal dispersion of copolymer has a polymer solids content from about 5 to about 60 weight percent and sufficient stabilizing ammonia to give the dispersion a pH of at least about 7.5. High solids dispersions are suitably prepared from lower solids dispersions by the method disclosed in the aforementioned patent to Moore et al.

In order to obtain a degree of sizing which is useful in manufacture of sized paper, it is necessary to utilize the copolymer sizing agent of the present invention in conjunction with any conventional retention aid which possesses cationic characteristics although it may not bear a cationic charge, herein called a cationic retention aid. These retention aids are useful as co-additives which enhance the retention of the copolymer sizing agent and which bring the copolymer sizing agent in closer proximity to the fibers of the cellulosic materials during the sizing operation.

Among the retention aids which may be employed are long chain fatty amines; polyamines such as polyalkylene polyamines including polyethylenimine and its derivatives; polyacrylamide; copolymers of ethylenimine with various monomers such as diethyl aminoethyl methacrylate; chromic sulfate; sodium alumate; aluminum sulfates (alum); animal glue; resins such as the reaction products of dibasic carboxylic acids, polyalkylene polyamines and epihalohydrins; reaction products of epihalohydrin and ammonia such as disclosed in U.S. Pat. No. 3,655,506 to Baggett including the reaction products of epihalohydrin and aliphatic polyamine having at least two amine hydrogens per molecule and reaction product of epihalohydrin and a mixture of ammonia and the polyamine as said reaction products are further described in U.S. Pat. No. 3,655,506 to Baggett which is hereby incorporated by reference in its entirety; polyamide polymers and copolymers such as polyamidechlorohydrin resins, vegetable gums, starch and modified starches such as oxidized starch and hydroxyethylated starches. Also of interest for use as retention aids are various cationic starch derivatives including primary, secondary, tertiary or quaternary amines, starch derivatives and other cationic nitrogen substituted starch derivatives, as well as cationic sulfonium and phosphonium starch derivatives. Preferred retention aids are the water-dispersible reaction products of epihalohydrin and ammonia and/or polyamine, including the reaction products of epihalohydrin and polyamine or mixture of polyamine and ammonia. Such reaction products have peak molecular weights as determined by gel permeation chromatography in the range from about 1000 to about 80,000, and comprise from about 0.9 to about 2.1 moles of epihalohydrin per mole of amine, i.e., ammonia, aliphatic polyamine or mixture of ammonia and polyamine.

In the internal sizing of paper and other cellulosic materials using the above-described copolymers as internal sizing agents, a number of variations and techniques may be employed. It is critical however, that all

of the techniques employed achieve uniform dispersal of the sizing agent throughout the cellulosic fiber during internal sizing. Uniform dispersal may be obtained by adding the ammoniated copolymer sizing agent in a fully dispersed form such as an aqueous colloidal dispersion. Any of the aforementioned retention aids may be added to the cellulosic fiber stock, e.g., the pulp slurry, either prior to, along with or after the addition of the ammoniated copolymer sizing agent. In order to achieve maximum distribution, it is preferable that the retention aid be added either subsequent to or simultaneously with the sizing agent.

Although order of addition of the ammoniated copolymer sizing agent and the retention aid is not critical, it is usually desirable, particularly when the retention aid is highly cationic or is a flocculant for the copolymer sizing agent, to add the copolymer sizing agent to the fiber stock prior to addition of the retention aid, simultaneously therewith or shortly thereafter, e.g., usually within 30 minutes. Preferably the copolymer sizing agent is added to the fiber stock slurry prior to addition of the retention aid. Whichever technique is chosen for the addition of the ammoniated copolymer and cationic retention aid to the fiber stock, care must be taken to avoid contact of the ammoniated copolymer and the retention aid prior to contacting the fiber stock.

The actual addition to the cellulosic material fiber of either the retention aid or the sizing agent may take place at any point in the cellulosic material manufacturing process prior to the ultimate conversion of wet-fibrous material into web, sheet or molded article. Thus, for example, in paper manufacture, the sizing agent may be added to the pulp while the latter is in the head box, beater, hydropulper or stock chest.

In order to obtain good internal sizing, it is desirable that the ammoniated copolymer sizing agents be uniformly dispersed throughout the fiber in as small a particle size as it is possible to obtain. One method for providing such uniform dispersions is to disperse the sizing agent in aqueous media prior to its addition to stock using, for example, a method as described hereinbefore. While it is generally desirable to use the ammoniated copolymer sizing agent in aqueous colloidal dispersion which is free of emulsifiers and surface active agents, such agents can be suitably employed in the practice of the invention provided that such agents are fugitive during sizing or otherwise do not impair the effectiveness of the copolymer sizing agent.

The sizing agents of this invention are most successfully utilized for the sizing of paper prepared from all types of both cellulosic and combination of cellulosic with non-cellulosic fibers. The cellulosic fibers which may most advantageously be used include the bleached and unbleached sulfate (kraft), bleached and unbleached sulfite, bleached and unbleached soda, neutral sulfite, semi-chemical, chemi-ground wood, ground wood and any combination of these fibers. These designations refer to wood pulp fibers which have been prepared by means of a variety of processes which are known in the pulp and paper industries.

It is understood that all types of additives such as pigments, fillers, stabilizers, retention aids, wet strength additives and dry strength additives, additional sizing agents, and the like may be employed in combination with the copolymer sizing agents of the present invention. Such additaments include kaolin clay, talc, tita-

nium dioxide, calcium carbonate, diatomaceous earth, plastic pigments, aluminum trihydrate, and precipitated silica.

The ammoniated copolymer sizing agents are suitably employed in amounts effective to achieve the purposes of the sizing such as water-resistance, i.e., an amount effective to size the cellulosic material. Generally, amounts ranging from about 0.03 to about 20 weight percent based on dry weight of the cellulosic material in the finished sheet or article are suitable, with preferred amounts being in the range from about 0.05 to about 2 weight percent and especially preferred amounts being in the range from about 0.2 to about 7 weight percent. It is understood that within this numerical range, the precise amount which is used will depend for the most part on the type of cellulosic material which is being employed, the specific operating conditions, as well as the particular end use for which the cellulosic material is destined. For example, paper which will require good water-resistance or ink holdout will necessitate the use of a higher concentration or sizing agent than a paper having characteristics which necessitate the use of only small amounts of sizing. Accordingly, any amount which is suitable to effect the desired end result of the sizing is suitable for the purpose of this invention.

These same factors also apply in relation to the amount of retention aid which is used in conjunction with ammoniated copolymer sizing agent. Thus, the skilled artisan will be able to use the retention aid and the sizing agent in any concentrations which is found to be applicable to the specific operating conditions of internally sizing cellulosic material as defined hereinbefore. However, as a general rule, the retention aid is usually employed in amount in the range from about 0.5 to about 8 weight parts per 1 weight part of copolymer sizing agent, preferably from about 1.5 to about 4 weight parts of retention aid per 1 weight part of copolymer sizing agent.

The following examples are given to illustrate the preferred embodiment of the invention and should not be construed as limiting its scope. In these examples, all parts and percentages are by weight unless otherwise noted.

#### EXAMPLE 1

A 500-g portion of ethylene/acrylic acid (87.3/12.7) copolymer having a number average molecular weight ( $M_n$ ) of 6950 is added to 240 ml of aqueous ammonia (28 percent  $NH_3$ ) in a 4 liter kettle containing 2.94 liters of water. The foregoing ingredients are stirred for 8 hours at 100°C, and the resulting dispersion is allowed to cool to room temperature. The dispersion is passed through gauze to remove flocculated material. The resulting filtrate is an aqueous dispersion containing 13.6 percent ethylene/ammonium acrylate copolymer solids and having pH of about 8.

A starch suspension is prepared by stirring 40 g of cationic starch\* in 400 g of water at 70°C

\*Potato starch bearing quaternary amino groups which is sold under the trademark "Sta-Lok 400" by A. E. Stanley Mfg. for 30 minutes. A 1-part portion of the aqueous dispersion of copolymer is stirred with 2.7 parts of the starch suspension for 5 minutes and diluted by addition of 33.8 parts of water. A 1-part portion of resulting combined dispersion is added to 236 parts of a 0.33 percent solids aqueous slurry of bleached sulfite pulp having a pH of 6.7 and processed in accordance with TAPPI T-200m-45. Handsheets are formed and dried in accordance with TAPPI T-205m-53. Surface wettability by water (angle of contact) of the handsheets (precured and cured) is determined and recorded in Table I.

As additional illustration of this embodiment, varying amounts of the combined aqueous dispersion of the copolymer and the cationic starch are used for internal sizing of the aforementioned pulp. In the foregoing manner, the treated pulp is converted to handsheets and tested for surface wettability. The results are also recorded in Table I.

TABLE I

| Sample No. | Additive Concentration lb/ton (1) |                 | Contact Angle With Water (2) |       |
|------------|-----------------------------------|-----------------|------------------------------|-------|
|            | Co-polymer                        | Cationic Starch | Pre-cured                    | Cured |
| 1          | 3                                 | 6               | 78°                          | 89°   |
| 2          | 6                                 | 12              | 86°                          | 101°  |
| 3          | 9                                 | 8               | 95°                          | 107°  |
| 4          | 12                                | 20              | 97°                          | 108°  |
| 5          | 15                                | 30              | 102°                         | 111°  |

(1) Measured in dry weights as pounds of specified additive per ton of pulp.

(2) Surface wettability by water (contact angle) before (pre-cured) and/or after (cured) curing as determined by TAPPI-458m-48.

(1) Measured in dry weights as pounds of specified additive per ton of pulp.

(2) Surface wettability by water (contact angle) before (pre-cured) and/or after (cured) curing as determined by TAPPI-458m-48.

#### EXAMPLE 2

In accordance with Example 1, portions of unbleached sulfite pulp having different pH values as shown in Table II are internally sized, formed into handsheets and tested for ink penetration. The results are recorded in Table II.

For purposes of comparison, several portions of unbleached sulfite pulp as described above are internally sized using a conventional rosin size as set forth in Table II, formed into handsheets and tested for ink penetration in a similar manner. The results which are recorded in Table II establish the copolymer to be a more effective sizing agent over a wider range of pH than the conventional rosin size. The results of ink penetration as recorded in Table II indicates the ability of the sized paper to resist penetration of ink applied to one side of the paper to the other. A higher value of percent reflectance indicates a higher resistance to penetration.

TABLE II

| Sample No. | Type               | Size                     |           | Retention Aid            |           |    | Ink Penetration, % reflectance at 120 sec. (2) |
|------------|--------------------|--------------------------|-----------|--------------------------|-----------|----|------------------------------------------------|
|            |                    | Concentration lb/ton (1) | Type      | Concentration lb/ton (1) | Beater pH |    |                                                |
| 1          | Et/AA( $NH_3$ )(a) | 12                       | Starch(b) | 22                       | 4.5       | 97 |                                                |
| 2          | Et/AA( $NH_3$ )(a) | 12                       | Starch(b) | 22                       | 6.5       | 93 |                                                |
| 3          | Et/AA( $NH_3$ )(a) | 12                       | Starch(b) | 22                       | 8.5       | 83 |                                                |
| 4          | Et/AA( $NH_3$ )(a) | 6.4                      | Starch(b) | 12                       | 5.5       | 81 |                                                |
| 5          | Et/AA( $NH_3$ )(a) | 7                        | Starch(b) | 13                       | 5.5       | 81 |                                                |
| 6          | Et/AA( $NH_3$ )(a) | 15                       | Starch(b) | 15                       | 5.5       | 81 |                                                |

TABLE II—Continued

| Sample No.       | Type     | Size                     |         | Retention Aid            |           |    | Ink Penetration, % reflectance at 120 sec. (2) |
|------------------|----------|--------------------------|---------|--------------------------|-----------|----|------------------------------------------------|
|                  |          | Concentration lb/ton (1) | Type    | Concentration lb/ton (1) | Beater pH |    |                                                |
| C <sub>1</sub> * | Rosin(c) | 40                       | Alum(d) | 80                       | 4.5       | 75 |                                                |
| C <sub>2</sub> * | Rosin(c) | 20                       | Alum(d) | 60                       | 4.5       | 50 |                                                |
| C <sub>3</sub> * | Rosin(c) | 15                       | Alum(d) | 30                       | 4.5       | 50 |                                                |
| C <sub>4</sub> * | Rosin(c) | 20                       | Alum(d) | 40                       | 5.75      | 71 |                                                |

\* Not an example of the invention.

(a) Ammoniated ethylene/acrylic acid copolymer described in Example 1.

(b) Cationic starch.

(c) Maleic anhydrides modified rosin.

(d) Aluminum sulfate (paper maker's grade).

(1) Same as in Table I.

(2) A photometric determination of black ink penetration through white or light-colored paper by measuring light reflectance on the side of the paper opposite to which a pool of the black ink is applied. The paper tested prior to inking using a black background of 0% reflectance has a 100% reflectance.

## EXAMPLE 3

In a manner similar to Example 2, bleached kraft pulp is internally sized with the copolymer of Example 1 and a variety of other sizes set forth in Table III, 20 formed into handsheets and tested for ink penetration. The results which are recorded in Table III show that the copolymer is a better sizing agent in terms of resistance to ink penetration under the prescribed conditions than the conventional sizes listed.

## EXAMPLE 4

In a manner similar to Example 2, bleached kraft hardwood pulp is internally sized with a copolymer of 58.5 percent ethylene and 41.5 percent ammonium acrylate. The internally sized pulp is formed into hand- 30

sheets and dried in accordance with TAPPI T-205m-53 and tested for surface wettability and ink penetration. The results are recorded in Table IV.

For the purposes of comparison, portions of an identical pulp are similarly sized with a copolymer of 54.7 percent ethylene and 45.3 percent sodium acrylate and a copolymer of 47.0 percent ethylene and 53.0 percent potassium acrylate. These comparative treated pulp slurries are formed into handsheets and dried in accordance with TAPPI T-205m-53 and tested for surface wettability and ink penetration. The results which are recorded in Table IV establish that the ammonium salt form of the copolymer is an effective sizing agent whereas alkali metal salt forms are not.

TABLE III

| Sample No.       | Type                       | Size                     |           | Retention Aid            |           |    | Ink Penetration, % reflectance at 120 sec. (2) |
|------------------|----------------------------|--------------------------|-----------|--------------------------|-----------|----|------------------------------------------------|
|                  |                            | Concentration lb/ton (1) | Type      | Concentration lb/ton (1) | Beater pH |    |                                                |
| 1                | Et/AA(NH <sub>3</sub> )(a) | 10.8                     | Starch(b) | 21.6                     | 4.5       | 93 |                                                |
| 2                | Et/AA(NH <sub>3</sub> )(a) | 8.6                      | Starch(b) | 17.2                     | 4.5       | 93 |                                                |
| 3                | ET/AA(NH <sub>3</sub> )(a) | 7.0                      | Starch(b) | 14.0                     | 4.5       | 88 |                                                |
| C <sub>1</sub> * | Poly(iminol stearate)      | 7.0                      | Starch(b) | 14.0                     | 4.5       | 90 |                                                |
| C <sub>2</sub> * | Poly(iminol stearate)      | 6.0                      | Starch(b) | 12.0                     | 4.5       | 86 |                                                |
| C <sub>3</sub> * | Poly(iminol stearate)      | 5.2                      | Starch(b) | 10.4                     | 4.5       | 80 |                                                |
| C <sub>4</sub> * | Poly(iminol stearate)      | 4.4                      | Starch(b) | 8.8                      | 4.5       | 50 |                                                |
| C <sub>5</sub> * | Rosin(c)                   | 20                       | Alum(d)   | 40                       | 4.5       | 87 |                                                |
| C <sub>6</sub> * | Rosin(c)                   | 15                       | Alum(d)   | 30                       | 4.5       | 70 |                                                |

\* Not an example of the invention.

(a)-(d) Same as in Table II.

(1)-(2) Same as in Table II.

TABLE IV

| Sample No.       | Type(a)                 | Size Concentration lb/ton (1) | Retention Aid Type | Concentration lb/ton (1) | Contact Angle With Water(2) |       | Ink Penetration, % Reflectance at 120 sec. (3) |
|------------------|-------------------------|-------------------------------|--------------------|--------------------------|-----------------------------|-------|------------------------------------------------|
|                  |                         |                               |                    |                          | Pre-cured                   | Cured |                                                |
| 1.               | Et/AA(NH <sub>3</sub> ) | 20                            | Polyamine(b)       | 10                       | 107                         | 116   | 88%                                            |
| 2                | Et/AA(NH <sub>3</sub> ) | 40                            | Polyamine(b)       | 10                       | 111                         | 116   | 99%                                            |
| A <sub>1</sub> * | Et/AA(Na)               | 20                            | Polyamine(b)       | 10                       | 82                          | 100   | 0                                              |
| A <sub>2</sub> * | Et/AA(Na)               | 40                            | Polyamine(b)       | 10                       | 98                          | 105   | 0                                              |
| B <sub>1</sub> * | Et/AA(K)                | 20                            | Polyamine(b)       | 10                       | 95                          | 101   | 0                                              |
| B <sub>2</sub> * | Et/AA(K)                | 40                            | Polyamine(b)       | 10                       | 102                         | 104   | 58%                                            |

\* Not an example of the invention.

(a) All sizes prepared from the same ethylene/acrylic acid (65.3/34.7) copolymer having a number average molecular weight of 4570.

(b) Polyalkylene polyamine.

(1) Same as (1) in Table II.

(2) Same as (2) in Table I.

(3) Same as (2) in Table II.

## EXAMPLE 5

A 500-g portion of ethylene/acrylic acid (87.3/12.7) copolymer having a melt flow viscosity [ASTM D-1238-65T(B)] using a plastometer having a 0.020 inch orifice] of 2 decig./min. (having a number average molecular weight of 6,950) is added to 240 mls. of aqueous ammonia (28 percent NH<sub>3</sub>) in a 4 liter kettle containing 2.94 liters of water. The foregoing ingredients are stirred for 8 hours at 100°C, and the resulting dispersion is allowed to cool to room temperature. The dispersion is passed through gauze to remove flocculated material. The resulting filtrate is an aqueous dispersion containing 13.6 copolymer solids.

An aqueous solution of a retention aid as specified in Table V is added in proportions specified in Table V to bleached kraft pulp slurry (0.33 percent solids in water) while stirring. The copolymer dispersion is added to the stirred pulp slurry in amount indicated in Table V. The pH of the pulp slurry is adjusted to 4.5 by adding sulfuric acid and the pulp slurry is formed into handsheet. The handsheet is tested for ink penetration and water contact angle and the results are recorded in Table V.

## EXAMPLE 6

A 7.3-lb. portion of ethylene/acrylic acid (86/14) copolymer having a melt flow viscosity (ASTM D-1238-65T(B) with a 0.020 inch orifice) of 2 decig./min. (number average molecular weight of 4,450) is added to 7.5 gallons of water and 0.617 gallons of aqueous ammonia (28% NH<sub>3</sub>) in a 10 gallon stirred kettle. The kettle is heated and stirred for three hours at 100°C and

45 psi. The product is drained and filtered through a 100 mesh stainless steel screen. A good amber colored dispersion having 10 percent copolymer solids is obtained.

- 5 A 4-part portion of the epichlorohydrin/ammonia reaction product as used in Example 5 (25 percent solids) is diluted with 27 parts of water. A 2.9-part portion of the foregoing copolymer dispersion is diluted with 4.8 parts of water. The two dilutions are added to 10 a bleached kraft pulp slurry. The mixture is adjusted to a pH of 3.5 with sulfuric acid. The pulp slurry is formed into a handsheet and tested for ink penetration and water contact angle. The foregoing procedure is repeated using pulp slurries adjusted to pH values of 4.8, 15 6.1, 7.1, 7.9, 9.1, and 10.2. The results of the foregoing tests which are recorded in Table VI show the copolymer sizing agent to be effective over a wide range of pH.

## EXAMPLE 7

- 20 A 40-g portion of ethylene/acrylic acid (89/11) copolymer having a melt flow viscosity (ASTM D-1,238-65T(B) with a 0.20 inch orifice) of 43 decig./min. (number average molecular weight of 4075) is added to 27 g. of aqueous ammonia (28 percent of NH<sub>3</sub>) and 25 200 g. of water in a 0.5 liter stainless steel bomb reactor. The bomb is sealed and the reaction mixture is shaken for 3 hours at 95°C. The resulting dispersion contains 15 percent copolymer solids.

- 30 A 0.18-part portion of an epichlorohydrin/ammonia reaction product as used in Example 5 (25 percent solids) is diluted with 6 parts of water. The resulting solution is added to a bleached kraft pulp slurry in the proportion set forth in Table VII and is stirred for one

TABLE V

| Sample No. | Copolymer Concentration lb/ton (1) | Retention Aid Type       | Concentration lb/ton (1) | Ink Penetration, % Reflectance at 120 sec. (2) | Contact Angle(3), precured |
|------------|------------------------------------|--------------------------|--------------------------|------------------------------------------------|----------------------------|
| 1          | 6                                  | PAPA(a)                  | 6                        | 93                                             | 95°                        |
| 2          | 6                                  | NH <sub>3</sub> /EPCH(b) | 15                       | 93                                             | 103°                       |
| 3          | 4                                  | NH <sub>3</sub> /EPCH(b) | 15                       | 70                                             | 105°                       |
| 4          | 1                                  | PEI(c)                   | 7.5                      | 83                                             | 90°                        |
| 5          | 2                                  | PEI(c)                   | 7.5                      | 97                                             | 115°                       |
| 6          | 4                                  | PAECHR(d)                | 15                       | 90                                             | 106°                       |

(a) Polyalkylene polyamine flocculant sold under the trademark "Purifloc C-31" by The Dow Chemical Co.

(b) Reaction product of epichlorohydrin/ammonia in the mole ratio of 1.7:1, said reaction product having molecular weight peaks at 5000 and 50,000 as measured by gel permeation chromatography.

(c) Polyethylenimine having a molecular weight of 600,000.

(d) Polyamide epichlorohydrin resin.

(1) Same as In Table I.

(2) Same as in Table II.

TABLE VI

| Sample No. | Additive Concentration(1), lbs/ton         |                                          | Ink Penetration, % Reflectance at 120 sec. (2) | Contact Angle, precured (3) | pH(4) |
|------------|--------------------------------------------|------------------------------------------|------------------------------------------------|-----------------------------|-------|
| Sample No. | Ethylene/Ammoniated Acrylic Acid Copolymer | Ammonia/Epichlorohydrin Reaction Product |                                                |                             |       |
| 1          | 10                                         | 15                                       | 98                                             | 115°                        | 3.5   |
| 2          | 10                                         | 15                                       | 98                                             | 120°                        | 4.8   |
| 3          | 10                                         | 15                                       | 99                                             | 117°                        | 6.1   |
| 4          | 10                                         | 15                                       | 99                                             | 118°                        | 7.1   |
| 5          | 10                                         | 15                                       | 100                                            | 122°                        | 7.9   |
| 6          | 10                                         | 15                                       | 95                                             | 120°                        | 9.1   |
| 7          | 10                                         | 15                                       | 98                                             | 118°                        | 10.2  |

(1) Same as in Table I.

(2) Same as in Table II.

(3) Same as (3) in Table V.

(4) pH of pulp slurry before processing into handsheets.

minute. A 0.19-part portion of the foregoing ethylene copolymer dispersion is diluted with 7.7 parts of water and is then added to the pulp slurry as an internal size in the proportion specified in Table VII. The pH of the

ammoniated copolymers are employed as sizing agents. The resultant handsheets are likewise tested for surface wettability and ink penetration. These results are also recorded in Table VIII.

TABLE VIII

| Sample No. | Type                                 | Size                                        |                                    | Retention aid                               |      | Beater pH | Contact angle, degrees <sup>2</sup> | Ink penetration <sup>3</sup> |
|------------|--------------------------------------|---------------------------------------------|------------------------------------|---------------------------------------------|------|-----------|-------------------------------------|------------------------------|
|            |                                      | Concen-<br>tration,<br>lb./ton <sup>1</sup> | Type                               | Concen-<br>tration,<br>lb./ton <sup>1</sup> | Type |           |                                     |                              |
| 1          | Et/AA(NH <sub>3</sub> ) <sup>a</sup> | 5                                           | NH <sub>3</sub> /EPCH <sup>d</sup> | 9                                           | 6.4  | 117       | 3,614                               |                              |
| A*         | Et/AA(NH <sub>3</sub> ) <sup>b</sup> | 5                                           | NH <sub>3</sub> /EPCH <sup>d</sup> | 9                                           | 6.65 | 60        | 0.9                                 |                              |
| 2          | Et/AA(NH <sub>3</sub> ) <sup>a</sup> | 10                                          | Sta-lok 400 <sup>e</sup>           | 20                                          | 6.25 | 84        | 6.0                                 |                              |
| B*         | Et/AA(NH <sub>3</sub> ) <sup>c</sup> | 10                                          | Sta-lok 400 <sup>e</sup>           | 20                                          | 6.2  | <20       | 0.1                                 |                              |

\*Not an example of the invention.

<sup>a</sup> Ammoniated ethylene/acrylic acid (86/14) copolymer having a number average molecular weight of 4,450.

<sup>b</sup> Ammoniated ethylene/acrylic acid (80.5/19.5) copolymer having a number average molecular weight of 30,000.

<sup>c</sup> Ammoniated ethylene/acrylic acid (80/20) copolymer having a melt flow viscosity [ASTM-D-1238-65 T(E)] of 250 decig./min. which approximately corresponds to a number average molecular weight of 18,300.

<sup>d</sup> Reaction product of epichlorohydrin/ammonia in a mole ratio of 1.61:1, said reaction product having molecular weight peaks at 2,500 and 65,000 as determined by gel permeation chromatography.

<sup>e</sup> Potato starch bearing quaternary amine groups as follows:



and manufactured by A. E. Staley Manufacturing.

<sup>1</sup> Same as in Table I.

<sup>2</sup> Same as (3) in Table V.

<sup>3</sup> Time in seconds taken for paper to have an 80% reflectance using test method (2) in Table II.

resulting pulp slurry is adjusted to 4.5 with sulfuric acid. The pulp is formed into a handsheet and is tested for ink penetration and water contact angle. The results are listed in Table VII.

30

What is claimed is:

1. In a method for internal sizing of a cellulosic material wherein an internal sizing agent and a retention aid are applied to the fibers of the cellulosic material, the

TABLE VII

| Sample No. | Ethylene Copolymer | Additive Concentration(1), lbs/ton | Ammonia/Epichlorohydrin Reaction Product | Ink Penetration, % Reflectance at 120 sec. (2) | Contact Angle, precured (3) |
|------------|--------------------|------------------------------------|------------------------------------------|------------------------------------------------|-----------------------------|
| 1          | 10                 | 15                                 |                                          | 91                                             | 112°                        |

(1) Same as in Table I.

(2) Same as in Table II.

(3) Same as (3) in Table V.

### EXAMPLE 8

Following the procedure of Example 5, an aqueous dispersion (11 percent copolymer solids) of ammoniated ethylene/acrylic acid (86/14) copolymer having a number average molecular weight of 4,450 is prepared.

An aqueous solution of a retention aid as specified in Table VIII is added in proportions specified in Table VIII to a bleached kraft pulp slurry (0.3 percent solids in water) while stirring. The ammoniated copolymer dispersion is then added to the stirred pulp slurry in the amount indicated in Table VIII. The pulp slurry is converted to handsheets and dried in accordance with TAPPI T-205m-53. Surface wettability by water (angle of contact) and ink penetration of the dried handsheets are then determined. The results are recorded in Table VIII.

For the purpose of comparison, the foregoing procedure is followed except that higher molecular weight

improvement wherein the internal sizing agent is a water-dispersible, water- and alkali-insoluble copolymer of an  $\alpha,\beta$ -ethylenically unsaturated hydrophobic monomer and an ammoniated  $\alpha,\beta$ -ethylenically unsaturated carboxylic acid, said copolymer having a number average molecular weight as determined by ebulliometry in the range from about 1,000 to about 10,000.

2. The improvement according to claim 1 wherein the cellulosic material is pulp.

3. The improvement according to claim 1 wherein the hydrophobic monomer is an  $\alpha,\beta$ -ethylenically unsaturated hydrocarbon.

4. The improvement according to claim 3 wherein the hydrocarbon is an aliphatic  $\alpha$ -monoolefin having 2 to 14 carbon atoms.

5. The improvement according to claim 4 wherein the aliphatic  $\alpha$ -monoolefin is ethylene.

6. The improvement according to claim 1 wherein the carboxylic acid is acrylic acid.

7. The improvement according to claim 1 wherein the carboxylic acid is methacrylic acid.
8. The improvement according to claim 5 wherein the copolymer is film-forming under the conditions of internal sizing.
9. The improvement of claim 8 wherein the copolymer has a number average molecular weight in the range from about 3000 to about 8000 and contains from about 10 to about 20 weight percent of  $\alpha,\beta$ -ethylenically unsaturated carboxylic acid.
10. The improvement according to claim 8 wherein the retention aid is the reaction product of ammonia and epihalohydrin.
11. The improvement of claim 10 wherein the reaction product has at least one molecular weight peak as determined by gel permeation chromatography in the range from about 2000 to about 70,000.
12. The improvement according to claim 8 wherein the retention aid is a cationic starch.
13. The improvement according to claim 8 wherein the retention aid is a polyalkylene polyamine.
14. The improvement according to claim 8 wherein the retention aid is polyethyleneimine.
15. The improvement according to claim 8 wherein the retention aid is a polyacrylamide.

16. The improvement according to claim 8 wherein the retention aid is a polyamideepichlorohydrin resin.
17. The improvement according to claim 1 wherein the cellulosic material is internally sized under conditions of pH of at least 7.
18. An internal sizing composition for a cellulosic material comprising a sizing amount of a water-dispersible, water- and alkali-insoluble copolymer of an  $\alpha,\beta$ -ethylenically unsaturated hydrophobic monomer and an ammoniated  $\alpha,\beta$ -ethylenically unsaturated carboxylic acid, said copolymer containing from about 6 to about 40 weight percent of the ammoniated carboxylic acid and having a number average molecular weight in the range from about 1,000 to about 10,000 and an amount of a retention aid effective to retain the copolymer on the cellulosic material.
19. The composition according to claim 18 wherein the retention aid is a cationic starch.
20. The composition according to claim 18 wherein the hydrophobic monomer is ethylene and the carboxylic acid is acrylic acid.
21. The composition of claim 18 wherein a reaction product of epihalohydrin and ammonia is the retention aid.

25

\* \* \* \* \*

30

35

40

45

50

55

60

65

UNITED STATES PATENT OFFICE  
CERTIFICATE OF CORRECTION

Patent No. 3,872,039 Dated March 18, 1975

Inventor(s) Walter Lee Vaughn et al

It is certified that error appears in the above-identified patent and that said Letters Patent are hereby corrected as shown below:

Cover page, fifth line down under the heading "Abstract", delete the space between the alpha and beta so that it reads -- $\alpha,\beta$ -ethylenically--.

Column 2, line 54, the word "of" should be --to--.

Column 3, line 35, the word "operations" should be --operation--.

Column 3, line 39, the word "dispersion" should be --dispersions--.

Column 3, line 61, the word "minimummm" should be --minimum--.

Column 8, lines 33-37, delete the footnotes (1) & (2), second occurrence, as they already appear directly under table.

Column 11, line 14, after the number "13.6", insert a percent sign so that it reads --13.6%--.

Column 11, Table V, the footnote (3) was not indicated beneath the table. This footnote should read as follows:

--(3) Same as (2) in Table I except that no determination is made subject to curing.--

Column 14, line 65, in Claim 5, the word "in" should be --is--.

Column 15, line 23, in Claim 14, the word "polyethyleneimine" should be --polyethylenimine--.

Column 16, line 15, in Claim 18, the word "effetive" should be --effective--.

Signed and Sealed this  
seventh Day of October 1975

[SEAL]

Attest:

RUTH C. MASON  
Attesting Officer

C. MARSHALL DANN  
Commissioner of Patents and Trademarks